

## 1

3,037,873  
METHOD AND COMPOSITION FOR  
COATING MOLDS

Frank Joseph Ingala, 3323 W. 64th Place, Chicago, Ill.  
No Drawing. Filed Apr. 4, 1960, Ser. No. 19,513  
5 Claims. (Cl. 106—38.23)

The present invention is directed to a method of and compositions for coating the inner surfaces of molds which are to receive molten metals at a high temperature. The invention is particularly applicable to the coating of metal molds employed for casting steel and other ferrous alloys.

When steel ingots are cast within a metal mold, molten steel is frequently splashed onto the sides of the mold during the pouring of the metal, and the splashed metal solidifies before the remainder of the ingot solidifies. This solidified metal on the sides of the mold may produce surface defects on the surface of the ingot which may manifest themselves as marks, slivers, or seams. The presence of these solidified deposits also gives rise to strains which tear the outer surface of the ingot during its solidification. In addition, the solidified splashed metal remains on the interior surfaces of the mold after the ingot has been stripped from the mold, thereby necessitating careful and time consuming cleaning and reconditioning of the mold prior to its reuse in another casting.

In the past, various means have been employed to provide an interface between the molten metal and the mold walls in order to minimize the adherence of molten metal splashes to the interior mold surfaces. Frequently, these mold coating compositions had taken the form of liquid coatings such as pitch or tar. However, this type of mold coating composition is necessarily limited in its applicability because at even relatively modest temperatures, the carbonaceous materials will tend to burn or become charred, resulting in the evolution of smoke and odors which are very objectionable. Furthermore, with the use of such materials, it was necessary to cool the mold substantially prior to pouring so that the coating would adhere to the inner surfaces of the mold.

Very substantial improvements in mold coating are achieved through the use of a dry process in which the constituents, in finely divided powder form are applied by means of a spray gun in a stream of air. The coating composition may be applied while the mold is at an elevated temperature so that it is not necessary to cool the mold further after stripping and prior to a second pouring.

In my previous Patent No. 2,578,976, issued December 18, 1951, I have described compositions which are particularly suitable for this use. Basically, the compositions there described consisted of a substantial proportion of a starch material, a resin, and a drying agent of a calcareous nature. While these compositions were very effective under ordinary conditions of use, they sometimes exhibited a tendency to create significant amounts of slag in the mold. It appears that this slag formation may have been due to the presence of the calcium in the compositions.

The present invention represents the distinct improvement upon the compositions and methods described in my aforementioned previous patent. With the compositions of the present invention, I can coat molds over a wider range of temperatures both higher and lower than previously. The principal reason for this is the fact that I include an improved low temperature binder in the new composition. More important, however, is the fact that the compositions of the present invention are stable at temperatures even beyond those which could be em-

## 2

ployed with the compositions of the previous invention, without the attendant difficulties of significant slag formation because the newly developed compositions are calcium free.

5 An object of the present invention is to provide an improved composition for coating the inner surfaces of molds to prevent adherence of splashed molten metal.

Another object of the present invention is to provide an improved method for coating the interior surfaces 10 of a mold over a wide temperature range.

Still another object of the invention is to provide an improved composition for coating metal molds which does not contribute slag forming ingredients to the molten metal contained in the mold.

15 A further object of the invention is to provide an improved method for application of mold coating compositions to hot molds.

In accordance with the present invention, I employ the combination of a starch material, a resinous bonding 20 agent, a bituminous composition, and talc in the form of a finely divided mixture.

The preferred compositions of the invention include starchy or farinaceous material containing less than about 15% moisture. Various starches can be employed, but

25 I prefer to employ potato starch, either alone, or in combination with other vegetable starches such as soy bean starch, tapioca starch, or corn starch. The principal function of the starch is to provide a film forming agent for the composition.

30 In order to achieve the maximum amount of adherence at relatively low temperatures, I prefer to include soy flour in the composition. As in the case of the starchy materials, the soy flour should contain no more than 15% moisture to function properly.

35 Additional low temperature binding effects are achieved through the inclusion of a resin or gum, particularly a light colored wood or gum rosin having a melting point of more than about 200° F.

Improved bonding at moderately elevated temperatures 40 is provided by adding the bituminous material, of which powdered pitch is the best example. A commercially available powdered pitch material having a melting point of about 250° C. (482° F.) is particularly preferred.

The talc is employed both as a refractory additive to 45 improve the high temperature behavior of the coating, and also as a drying agent to permit the storage of the coating composition without caking or lumping.

The relative percentages of the various degrees of the 50 composition, together with the range of particle sizes employed for each, is given in the following table:

| Ingredient               | Particle size        | Percent by weight |
|--------------------------|----------------------|-------------------|
| 55 Starch.....           | 200 to 400 mesh..... | 30-60             |
| Soy flour.....           | 200 to 250 mesh..... | 10-30             |
| Resin.....               | 150 to 400 mesh..... | 15-35             |
| Bituminous material..... | 150 to 400 mesh..... | 10-20             |
| Talc.....                | 200 to 400 mesh..... | 5-10              |

60 For best results, it is important that the total moisture content of the composition not exceed 8% by weight.

The ingredients are blended into the sprayable composition by thoroughly blending the dry ingredients, and then passing the mixture through a 150 mesh screen. The material may then be applied to the interior surfaces 65 of an ingot mold or the like by blowing the composition in powdered form under a positive air pressure into the mold. When the composition contacts the heated mold wall, the binder ingredients melt or soften to adhere to the wall and bind the remaining of the solids to the surface. With the types of compositions indicated above, I have successfully supplied coatings on mold surfaces

having temperatures as high as 950° F. although it is preferable, if possible, to work on a mold which has a temperature of about 700 to 750° F. because adherence is at its best in this temperature range.

The following specific examples illustrate the types of formulae coming within the scope of the invention and the results achieved:

*Example I*

A coating composition containing the following ingredients was prepared:

|                                                | Percent |
|------------------------------------------------|---------|
| Potato starch (11½% moisture), 200 to 400 mesh | 20      |
| Corn starch (7½% moisture), 200 to 400 mesh    | 20      |
| Wood rosin, 150 to 300 mesh                    | 30      |
| Soy flour (12% moisture), 200 to 250 mesh      | 15      |
| Powdered pitch, 150 to 400 mesh                | 10      |
| Talc, 400 mesh                                 | 5       |

These ingredients were mixed until they were well blended and then passed through a screen of 150 mesh. The composition was applied to the mold surfaces of an ingot mold in a current of air, the mold being at a temperature of about 700° F. Molten steel was poured into the mold and cooled to form the ingot. When the ingot was stripped from the mold, there was a substantial decrease in surface defects than ordinarily occurred in the same mold, and the mold itself had clean wall surfaces.

*Example II*

A slightly modified composition was prepared from the following ingredients:

|                                               | Percent |
|-----------------------------------------------|---------|
| Potato starch (11% moisture), 200 to 400 mesh | 35      |
| Soy flour (12% moisture), 200 to 250 mesh     | 25      |
| Wood rosin, 150 to 300 mesh                   | 20      |
| Powdered pitch, 150 to 400 mesh               | 15      |
| Talc, 400 mesh                                | 5       |

The foregoing composition was particularly effective in coating molds which had a lower surface temperature. As in the case of the material of Example I, the ingot was stripped from the mold cleanly, and the mold itself remained clean.

*Example III*

A metal mold was coated with the following composition:

|                                               | Percent |
|-----------------------------------------------|---------|
| Potato starch (11% moisture), 200 to 400 mesh | 50      |
| Soy flour (12% moisture), 200 to 250 mesh     | 20      |
| Wood rosin, 150 to 400 mesh                   | 10      |
| Powdered pitch, 150 to 400 mesh               | 15      |
| Talc                                          | 5       |

A steel ingot solidified in the mold coated with the foregoing composition was easily stripped from the mold without significant surface defects, and without impairing the surface of the mold.

*Example IV*

Another mold for casting steel ingots was coated with the following composition:

|                                               | Percent |
|-----------------------------------------------|---------|
| Potato starch (11% moisture), 200 to 400 mesh | 30      |
| Soy flour (10½% moisture), 200 to 350 mesh    | 30      |
| Wood rosin, 150 to 350 mesh                   | 20      |
| Powdered pitch, 150 to 250 mesh               | 15      |
| Talc                                          | 5       |

The finely divided mixture was sprayed by means of a conventional spray gun in a current of air onto the inner surfaces of a metal mold used for casting steel. The ingot which resulted was stripped from the mold without difficulty and the mold surfaces were clean after the stripping. No evidence of additional slag formation was

determined due to the presence of the coating composition.

It will be evident that various modifications can be made to the described embodiments without departing from the scope of the present invention.

I claim as my invention:

1. A dry, finely divided, air transportable composition for coating the inner surfaces of a mold comprising a finely divided mixture containing the following ingredients:

|           | Percent by weight |
|-----------|-------------------|
| Starch    | 30 to 60          |
| Soy flour | 10 to 30          |
| Rosin     | 15 to 35          |
| Pitch     | 10 to 20          |
| Talc      | 5 to 10           |

2. A dry, finely divided, air transportable composition for coating the inner surfaces of a mold comprising a finely divided mixture containing the following ingredients:

|           | Percent by weight |
|-----------|-------------------|
| Starch    | 30 to 60          |
| Soy flour | 10 to 30          |
| Rosin     | 15 to 35          |
| Pitch     | 10 to 20          |
| Talc      | 5 to 10           |

said composition containing no more than 8% by weight of moisture.

3. A dry, finely divided, air transportable composition for coating the inner surfaces of a mold comprising a finely divided mixture containing the following ingredients:

|                             | Percent by weight |
|-----------------------------|-------------------|
| Starch (200 to 400 mesh)    | 30 to 60          |
| Soy flour (200 to 250 mesh) | 10 to 30          |
| Rosin (150 to 400 mesh)     | 15 to 35          |
| Pitch (150 to 400 mesh)     | 10 to 20          |
| Talc (200 to 400 mesh)      | 5 to 10           |

4. The method of coating the inner surfaces of a mold having a surface temperature of up to 950° F. which comprises blowing against said surface an air stream carrying a finely divided mixture having the following composition:

|           | Percent by weight |
|-----------|-------------------|
| Starch    | 30 to 60          |
| Soy flour | 10 to 30          |
| Rosin     | 15 to 35          |
| Pitch     | 10 to 20          |
| Talc      | 5 to 10           |

until an appreciable coating of said mixture appeared on said surface.

5. The method of coating the inner surfaces of a mold having a surface temperature of up to 950° F. which comprises blowing against said surface an air stream carrying a finely divided mixture having the following composition:

|           | Percent by weight |
|-----------|-------------------|
| Starch    | 30 to 60          |
| Soy flour | 10 to 30          |
| Rosin     | 15 to 35          |
| Pitch     | 10 to 20          |
| Talc      | 5 to 10           |

moisture not more than 8%, until an appreciable coating of said mixture appears on said surface.

**References Cited in the file of this patent**

**UNITED STATES PATENTS**

|           |         |               |
|-----------|---------|---------------|
| 2,476,933 | Wallace | July 19, 1949 |
| 2,578,976 | Ingala  | Dec. 18, 1951 |

**FOREIGN PATENTS**

|        |               |         |
|--------|---------------|---------|
| 14,571 | Great Britain | of 1893 |
|--------|---------------|---------|